

## UNITED STATES PATENT OFFICE

1,932,867

## ALUMINUM ALLOYS

Robert T. Wood, Cleveland, Ohio, assignor to  
Aluminum Company of America, Pittsburgh,  
Pa., a corporation of Pennsylvania

No Drawing. Original application September 21,  
1932, Serial No. 634,155. Divided and this ap-  
plication November 30, 1932. Serial No.  
645,121

## 1 Claim. (Cl. 75—1).

This invention relates to aluminum base al-  
loys containing magnesium. The invention has  
for its object the improvement of alloys of this  
class by the addition thereto of about 0.05 to  
2.0 per cent by weight of calcium. The invention  
is particularly concerned with the specific  
alloys hereinafter described.

The claim of this application covers certain  
matter divided from my copending application  
Serial No. 634,155 which is, in part, a continuation  
of my copending application Serial No.  
595,231. Inventions disclosed but not claimed  
herein are claimed in my copending applica-  
tions Serial Nos. 595,231, filed February 25, 1932,  
645,108 to 645,120 inclusive, and 645,122 to  
645,125 inclusive, all filed November 30, 1932.

Considerable difficulty has heretofore been en-  
countered in attempts to commercially produce  
castings of aluminum base alloys containing  
substantial amounts of magnesium. This diffi-  
culty is encountered both in the making of sand  
castings and permanent mold or chill-mold cast-  
ings, although the nature of the difficulty differs  
somewhat in each case. In the case of sand  
castings there occurs a reaction between the  
molten aluminum base alloy containing mag-  
nesium and the ordinary sand-mold materials,  
or vapors generated therefrom. There is also  
a reaction with the atmosphere. In addition,  
the magnesium-containing aluminum base alloy  
does not flow freely through narrow mold sec-  
tions at ordinary pouring temperatures and, if  
the pouring temperature be raised, the solidified  
alloy is unsound. If the aluminum base alloy  
containing magnesium be cast in a chill-mold  
the reaction effect is minimized to some extent,  
but the troubles arising from cold-shuts and  
mis-runs are accentuated because of the more  
rapid chilling of the molten metal. The con-  
siderations apply to the aluminum base alloys  
specifically disclosed herein and particularly to  
such alloys.

I have discovered that when calcium is added  
to aluminum base alloys of the type and compo-  
sition herein described, these difficulties are, to  
a considerable extent, eliminated. The calcium  
should be present in amounts ranging from 0.05  
per cent to 2.0 per cent by weight subject to  
specific considerations as hereinafter disclosed.  
In the melting of aluminum alloys of the com-  
positions herein described, a viscous scum often  
forms at the surface of the molten metal. Fail-  
ure of the molten metal to run properly through  
narrow mold apertures is caused, in part, by  
shreds or particles of this scum being suspended

in the molten metal and offering a resistance  
to the free passage of the metal through the  
apertures. Regardless of the cause of this low  
fluidity, I have discovered that the addition to  
the alloy of relatively small amounts of calcium,  
in the preferred range between 0.05 to 0.5 per  
cent, improves the casting characteristics to a  
very considerable extent and simultaneously ef-  
fects a reduction of the scum or dross collecting  
at or near the surface. In the casting of articles  
in sand molds, I prefer to add calcium in  
amounts less than about 0.5 per cent except in  
instances where some reduction of tensile  
strength or other mechanical or tensile property  
is immaterial. In amounts of more than 0.5  
per cent the calcium addition produces the ad-  
vantages enumerated herein but has a tendency  
to lower some of the physical properties of the  
alloys. This effect is not harmful when calcium  
is present in amounts of about 0.5 per cent or  
less, but when high strength is not a desidera-  
tum the calcium may be used in amounts up  
to about 2.0 per cent. In intricate permanent  
mold castings, where casting troubles are very  
serious if no calcium be added, the improved  
physical properties obtained coincident with the  
production of good castings more than offset  
the diminution in properties which might other-  
wise result from the use of the calcium.

I have also discovered that when calcium is  
added to aluminum base alloys containing mag-  
nesium, the amount of gas evolved during solidi-  
fication of the alloys is considerably reduced.  
When from about 0.05 per cent to 2.0 per cent  
by weight of calcium is added to the alloys, the  
amount of gas evolved becomes less marked  
with increasing calcium content and the reduc-  
tion of gas evolution may be so marked that the  
molten metal cools to the solidification tempera-  
ture with a smooth mirror-like surface. I prefer  
to restrict the amount of calcium added to 2.0  
per cent or less since above this amount the  
physical properties of the alloys may be too seri-  
ously affected. If the best physical properties  
are desired with an improved, although not com-  
plete, degree of gas prevention, I keep the cal-  
cium content of the alloys between 0.05 per  
cent and about 0.5 per cent.

In the application of the principles of my in-  
vention I have determined that certain alumi-  
num base alloys containing magnesium are par-  
ticularly benefited thereby. For example, a  
very useful aluminum base alloy is one contain-  
ing about 2.0 to 9.0 per cent of magnesium and  
0.05 per cent to 2.0 per cent of calcium, as is

also aluminum base alloy containing about 2.0 to 15.0 per cent of magnesium, 0.1 to 3.5 per cent of cobalt, and 0.05 to 2.0 per cent of calcium to which other elements such as copper, antimony, bismuth, nickel, manganese, and other well known alloying elements may be added to produce particular properties therein.

Likewise is the addition of 0.05 to 2.0 per cent of calcium beneficial to those aluminum base alloys which contain about 2.0 to 15.0 per cent of magnesium and 0.05 to 0.4 per cent of at least one of the class of metals here defined as antimony and bismuth, such alloys being very useful where use at high temperatures is contemplated. Calcium may likewise be added to improve such alloys when they contain, in addition to magnesium and antimony and/or bismuth, one or more of such alloying elements as cobalt, copper, nickel, manganese, zinc, etc. which may be added to modify or produce a specific property in the alloy.

The addition of 0.05 to 2.0 per cent of calcium is very beneficial in the case of a series of aluminum base alloys which contain as major alloying elements about 2.0 to 10.0 per cent of magnesium and about 0.2 to 5.0 per cent of nickel. For instance, an aluminum base alloy containing 3.0 to 7.5 per cent of magnesium and 0.2 to 2.0 per cent of nickel is improved by the addition of 0.05 to 2.0 per cent of calcium as is, likewise, this same alloy when it also contains about 0.05 to 0.4 per cent of one or more of the class of elements composed of antimony and bismuth. Another excellent aluminum base alloy prepared in accordance with the principles of my invention is one containing 3.0 to 8.0 per cent of magnesium, 0.5 to 4.0 per cent of nickel, 0.5 to 4.0 per cent of manganese, and 0.05 to 2.0 per cent of calcium, which alloy may also be improved, particularly for application at high temperatures, by the addition of 0.05 to 0.4 per cent of at least one of the class of elements composed of antimony and bismuth.

The principles of my invention find particular application in the case of aluminum base alloys containing magnesium, nickel, and chromium, and aluminum base alloys containing magnesium, nickel and copper, as well as those alloys containing magnesium, nickel, and cobalt. Examples may be given of aluminum base alloys containing 2.0 to 10.0 per cent of magnesium, 0.2 to 5.0 per cent of nickel, 0.5 to 3.5 per cent of chromium, and 0.05 to 2.0 per cent of calcium. An aluminum base alloy containing 3.0 to 8.0 per cent of magnesium, 0.5 to 3.5 per cent of nickel, 0.5 to 3.5 per cent of chromium, and 0.05 to 2.0 per cent of calcium has excellent casting properties and the high temperature properties of this alloy can be favorably affected by the addition of 0.05 to 0.4 per cent of at least one of a class of elements composed of bismuth and antimony. Examples may be given of aluminum base al-

loy containing 2.0 to 10.0 per cent of magnesium, 0.2 to 5.0 per cent of nickel, 1.0 to 6.0 per cent of copper, and 0.05 to 2.0 per cent of calcium. An excellent alloy of this type is one containing 3.0 to 8.0 per cent of magnesium, 0.5 to 5.0 per cent of nickel, 1.0 to 6.0 per cent of copper, and 0.05 to 2.0 per cent of calcium with or without 0.05 to 0.4 per cent of at least one of the class of elements composed of antimony and bismuth and with or without the further addition of 0.5 to 3.5 per cent of at least one of a class of elements composed of cobalt and chromium, and with or without the further addition of 0.1 to 1.0 per cent of at least one of a class of elements composed of tungsten, vanadium, molybdenum, titanium, and zirconium.

Other excellent alloys are those aluminum base alloys containing about 2.0 to 10.0 per cent magnesium, 0.2 to 5.0 per cent nickel, 0.1 to 3.5 per cent cobalt, and 0.05 to 2.0 per cent of calcium. A particular example of this class of alloys, which may also contain with considerable advantage 0.05 to 0.4 per cent of a class of elements composed of antimony and bismuth, is the aluminum base alloy containing 3.0 to 8.0 per cent magnesium, 0.5 to 4.0 per cent nickel, 0.1 to 3.0 per cent cobalt, and 0.05 to 2.0 per cent calcium.

Among other magnesium-containing aluminum base alloys which I have found to be particularly benefited by the presence of calcium are numbered the aluminum base alloys containing 3.0 to 8.0 per cent of magnesium, 1.0 to 6.0 per cent of copper, 0.5 to 3.5 per cent of chromium, and 0.05 to 2.0 per cent of calcium, with or without the addition of 0.05 to 0.4 per cent of at least one of a class of metals composed of antimony and bismuth and with or without the addition of other alloying elements.

The alloys herein described may be produced by the usual methods of alloying metals. The calcium is preferably added to the molten alloy by thrusting the calcium beneath the surface with tongs or other suitable instrument. The aluminum used in preparing the alloys may be pure or it may contain the impurities found in commercial grades of this metal. Ordinarily a good commercial grade of virgin aluminum will give excellent results and is preferable.

Having thus explained and described my invention, I claim:

A metallic alloy consisting of 3.0 to 8.0 per cent by weight of magnesium, 0.5 to 3.5 per cent by weight of chromium, 0.05 to 0.4 per cent by weight of at least one of a class of elements composed of antimony and bismuth, 1.0 to 6.0 per cent by weight of copper, and 0.05 to 2.0 per cent by weight of calcium, the balance being aluminum.

ROBERT T. WOOD.